

# United States Patent Office

2,824,837  
Patented Feb. 25, 1958

1

2,824,837

## SOAP-SALT COMPLEX GREASE CONTAINING n-ACYL p-AMINOPHENOL

Arnold J. Morway, Rahway, N. J., assignor to Esso Research and Engineering Company, a corporation of Delaware

No Drawing. Application April 30, 1954  
Serial No. 426,927

12 Claims. (Cl. 252—40.7)

This invention relates to improved lubricating grease compositions having suitable characteristics for operation at elevated temperatures. In particular, the instant invention relates to lubricating grease compositions having outstanding high temperature properties which comprise complex alkaline earth soap greases wherein the soap system consists of a combination of the soap of high and low molecular weight fatty acids, the low molecular weight acid predominating, which contains combined therein a minor but stabilizing proportion of an n-acyl p-aminophenol.

High temperature lubricating grease compositions which are prepared by thickening a lubricating oil with a complex soap-salt system wherein the salt component predominates have been described in the art. However, these excellent high temperature lubricating grease compositions tend to harden excessively on storage. There first appears on the surface of these complex greases a hard crust which gradually extends throughout the body of the grease. It has been proposed to eliminate this crust formation and hardening effect by the incorporation of minor amounts of hydroxy fatty acids such as the mono- or di-hydroxy stearic acids, hydrogenated castor oil and the like.

It has now been found and forms the object of this invention that the tendency to harden noted in these soap-salt complex greases may be substantially eliminated by the inclusion in the grease composition of minor amounts of a class of compounds referred to as the n-acyl p-aminophenols, to be more completely described below.

The following series of examples illustrate the inventive concept.

## EXAMPLES 1 AND 2

| Formulation                         | Example 1—<br>Percent<br>Weight | Example 2—<br>Percent<br>Weight |
|-------------------------------------|---------------------------------|---------------------------------|
| Ingredients:                        |                                 |                                 |
| Hydrogenated Fish Oil Acids         | 2.0                             | 4.0                             |
| N-stearyl-p-aminophenol             | 2.0                             | None                            |
| Glacial acetic acid                 | 8.0                             | 8.0                             |
| Hydrated lime                       | 5.4                             | 6.0                             |
| Phenyl alpha-naphthylamine          | 0.5                             | 0.5                             |
| Naphthenic distillate SUS @ 210° F. | 55                              |                                 |
| Mol Ratio (Acetic: Hydrofol Acid)   | 82.1                            | 81.5                            |
|                                     | 19:1                            | 10:1                            |

*Preparation.*—The oil, lime and Hydrofol acid are charged to a fire heated kettle and warmed to 135° F., at which time the acetic acid is charged. The temperature is then raised to 500° F., and the grease cooled while stirring to 300° F. The n-stearyl p-aminophenol is added and the grease cooled to 250° F. where the phenyl alpha-naphthylamine is charged and the grease further cooled to 200° F. The grease is then homogenized and filtered. Comparative data are set out in Table I below.

2  
Table I

|    | Properties                                                           | Example 1                           | Example 2 |
|----|----------------------------------------------------------------------|-------------------------------------|-----------|
| 5  | Appearance                                                           | Excellent, smooth, uniform products |           |
|    | Penetration 77° F. mm./10:                                           |                                     |           |
|    | Unworked                                                             | 200                                 | 195       |
|    | Worked 60 strokes                                                    | 297                                 | 238       |
|    | Worked 100,000 strokes                                               | 295                                 | 308       |
|    | Dropping Point                                                       | None                                | None      |
| 10 | Wheel Bearing Test: 6 hours at 220° F.                               | Pass (no leakage)                   | Pass      |
|    | Norma-Hoffman Oxidation: Hours to 5 p. s. i. drop in oxygen pressure | 1 468                               | 320       |
|    | Penetration after 1 week storage:                                    |                                     |           |
|    | Unworked                                                             | 205                                 | 185       |
|    | Worked 60 strokes                                                    | 291                                 | 216       |
|    | Penetration after 3 months' storage:                                 |                                     |           |
| 15 | Unworked                                                             | 199                                 | 120       |
|    | Worked 60 strokes                                                    | 288                                 | 155       |

<sup>1</sup> With no phenyl alpha-naphthylamine present in composition on the same test, the time (hours) to a 5 p. s. i. drop in oxygen pressure was 468 hours.

<sup>2</sup> Heavy crust on grease.

It will be noted that the inclusion of the n-stearyl p-aminophenol in the grease composition of Example 1 completely eliminates the crust formation which was found to exist in Example 2. It is also to be noted that when the phenyl alpha-naphthylamine was omitted from Example 1, the Norma-Hoffman oxidation test gave the same results showing that the n-stearyl p-aminophenol served a dual function.

## EXAMPLES 3 AND 4

| Formulation (percent weight)            | Example 3 |      | Example 4 |      |
|-----------------------------------------|-----------|------|-----------|------|
|                                         | a         | b    | a         | b    |
| N-lauroyl p-aminophenol                 | 2.0       | none | 1.0       | none |
| Hydrogenated fish oil acids             | 2.0       | 2.0  | 3.0       | 4.0  |
| Glacial acetic acid                     | 8.0       | 8.0  | 8.0       | 8.0  |
| Hydrated lime                           | 5.5       | 6.0  | 5.8       | 6.0  |
| Naphthenic distillate (55 SUS/ 210° F.) | 82.5      | 84.0 | 82.2      | 82.0 |
| Mol ratio (Acetic: Hydrofol Acids)      | 19:1      | 19:1 | 13:1      | 10:1 |

*Preparation.*—Charged oil, fatty acids and lime to a fire heated kettle and warmed while agitating to 130° F. Then added the acetic acid and continued heating to 500° F. Cooled while agitating to 300° F. Added N-lauroyl p-aminophenol and cooled to 200° F. The grease was homogenized and filtered. Comparative data are set out in Table II below.

## Table II

| Properties                                                            | Example 3                  |      | Example 4 |      |
|-----------------------------------------------------------------------|----------------------------|------|-----------|------|
|                                                                       | a                          | b    | a         | b    |
| Percent free alkalinity (as NaOH)                                     | 0.08                       | 0.42 | 0.32      | 0.21 |
| Appearance                                                            | Excellent, smooth, uniform |      |           |      |
| Penetrations 77° F. mm./10:                                           |                            |      |           |      |
| Unworked                                                              | 255                        | 217  | 202       | 195  |
| Worked 60 strokes                                                     | 289                        | 242  | 258       | 238  |
| Worked 100,000 strokes                                                | 300                        | 330  | 295       | 308  |
| Wheel Bearing Test: 6 hours at 220° F.                                | Pass (no leakage)          |      |           |      |
| Norma-Hoffman Oxidation: Hours to 5 p. s. i. drop                     | 372+                       | 34   | 345       | 26   |
| A.F.B.M.A.-N.L.G.I. Lubrication Life Test: 10,000 R. P. M. at 250° F. | 556                        | 610  | 432       | 527  |
| Dropping Point, °F.                                                   | None                       | None | None      | None |
| Penetration after 1 week storage:                                     |                            |      |           |      |
| Unworked                                                              | 252                        | 200  | 200       | 185  |
| Worked 60 strokes                                                     | 263                        | 220  | 259       | 216  |
| Penetration after 3 months storage:                                   |                            |      |           |      |
| Unworked                                                              | 250                        | 145  | 199       | 120  |
| Worked 60 strokes                                                     | 270                        | 159  | 265       | 150  |

<sup>1</sup> Heavy crust formation on grease surface.

When the data on oxidation life and structure after storage is examined the advantage of incorporation of the N-acyl p-aminophenol becomes quite apparent (Examples 3a and 4a versus Examples 3b and 4b).

The N-acyl aminophenols incorporated in the grease compositions of this invention have the following general formula:



wherein R is an alkyl group containing from 10 to 22 carbon atoms and wherein R' and R'' are hydrogen atoms or alkyl groups containing from 1 to 20 carbon atoms.

The preferred embodiment of this invention contemplates the use of compounds, according to the formula above, wherein R' and R'' are hydrogen atoms and wherein R is a straight chain aliphatic group containing from 12 to 22 carbon atoms. Exemplary of these preferred compounds are N-lauroyl p-aminophenol, N-palmitoyl p-aminophenol, N-stearoyl p-aminophenol, N-arachidoyl p-aminophenol and N-behenoyl p-aminophenol. N-lauroyl p-aminophenol, N-stearoyl and N-palmitoyl p-aminophenol or mixtures of these are especially preferred.

The alkylated acyl p-aminophenols exemplified by the formula above when R' and R'' are alkyl groups containing from 1 to 20 and preferably from 4 to 15 carbon atoms, are also operable. Compounds such as N-n-valeryl-4-amino-3-pentadecyl phenol, (N-n-pentanoyl-4-amino-3-pentadecyl phenol), N-n-propanoyl-4-amino-3-pentadecyl phenol, N-n-pentanoyl-4-amino-2,6-di-tert-butyl phenol, N-n-hexyl-4-amino-2-hexyl phenol, are examples of the alkylated acyl p-aminophenols which are operable. The iso compounds, such as those obtained from Oxo acids, are also contemplated.

The preparation of these acyl p-aminophenols is accomplished by simply admixing the desired acid with the desired p-aminophenol and heating the mixture under proper reaction conditions. The reaction progresses smoothly (splitting off water) giving the desired acyl p-aminophenol which may be purified by any of the various methods known to the art such as distillation, crystallization, extraction, etc.

The high metal content soap salt complexes containing the metal salt of at least 7 mols of a low molecular weight carboxylic acid for each mol of saponified high molecular weight acid as described above may be incorporated into a wide variety of lubricating oils either naturally occurring or of synthetic origin. These soap complexes may be combined with mineral or synthetic lubricating oils in grease making proportion, that is to say, containing from 5 to 30 weight percent of the complex soap.

The high molecular weight acids useful for the purposes of the present invention are those having 12-30 carbon atoms and preferably those having 14-22 carbon atoms per molecule. These acids may be derived from saturated or unsaturated naturally occurring or synthetic fatty materials. The fatty acids normally used in the manufacture of conventional greases, particularly the more saturated acids, are preferred. Examples of such acids include stearic, hydroxy stearic, such as 12-hydroxy stearic, di-hydroxy stearic, poly-hydroxy stearic and other saturated hydroxy fatty acids, arachidic, hydrogenated fish oil and tallow acids, etc. Unsaturated acids, such as oleic, ricinoleic and similar acids may likewise be used.

Suitable low molecular weight acids include saturated and unsaturated aliphatic monocarboxylic acids having about 1-6 carbon atoms, such as formic, acetic, propionic, furoic, acrylic, and similar acids including their hydroxy derivatives, such as lactic acid, etc. Formic and, particularly, acetic acid are preferred.

The choice of the metal component depends to a certain extent on the use for which the complex soap of the

invention is contemplated. The alkaline earth metals, particularly calcium, strontium, barium and magnesium are useful for many purposes of the invention. These metals afford greatest advantages when used as thickeners in the manufacture of greases because they permit the production of greases having outstanding load-carrying characteristics and satisfactory structural stability at high temperatures and under mechanical stress even without the use of conventional extreme pressure and stabilizing agents. The alkaline earth metals differ in this respect from the alkali metals. Complex soaps of high alkali metal content, which are analogous to soap-salt complexes of the present invention regarding type and mol ratio of the acids used, yield greases of poorer structural stability, even when added to the oil dispersant in relatively high proportions.

The high metal content soap-salt complexes of the invention may be prepared by coneutralization of a mixture of the high and low molecular weight acids with suitable bases, particularly the hydroxide and/or carbonates of the metals desired. This coneutralization step may be carried out in situ in the liquid menstruum to which the complex soap is to be applied in actual use. For example, the mixed acids may be coneutralized in a portion or all of the lubricating oil forming the dispersant of a grease to be thickened by the complex soap. Similarly, the coneutralization may be carried out in fuel oil or other dispersant or solvent fluids. Coneutralization is particularly desirable in cases in which the soap and salt have the same metal constituent. Usually the coneutralized material is heated to high temperatures of about 450°-550° F. or higher, prior to use, to dehydrate the product and to promote formation of the complex. When this heating step is carried out in a liquid dispersant the latter should have a boiling point above the heating temperature of the heat treatment and the heating step should be carried out under pressure.

Instead of using high molecular weight fatty acids proper, esters thereof, particularly the glycerides or other acidogenic materials such as the nitriles, may serve as the starting materials. Naturally occurring animal or vegetable fats and oils are preferred materials of this type. Also, the low molecular weight carboxylic acids may be employed in the form of suitable esters, such as those of glycerine, ethanol, etc., or other acidogenic compounds, such as the nitriles. Conventional conditions conducive to the saponification of these esters followed by dehydration and alcohol removal may be used. Esters of this type may be used as described in the case of coneutralization as well as in the case of separate formation of the soap and salt described below.

The high metal content soap-salt complexes of the invention may also be prepared by separately preforming at least a portion of the high molecular weight acid soap and/or the low molecular weight carboxylic acid salt and intimately mixing the soap with the salt, followed by heating, if necessary. This method is useful particularly when different metals are employed as bases for the soap and salt constituents respectively.

The choice of the material to which the high metal content complex soaps of the invention are applied depends, of course, on the use contemplated. For grease manufacture, in accordance with the invention, mineral as well as synthetic lubricating oils may be used including well-known di-esters, complex esters, hydrocarbon polymers, silicone oils, polyglycol derivatives, etc. Quite generally, these oils should have a viscosity within the range of about 35-200 SUS at 210° F. and flash points of about 350°-600° F. A viscosity index of 100 or higher may be employed; however, oils of lower viscosity index, such as below 60 V. I. give better yields. It has also been found that soap-salt complexes containing more than 30 mols, e. g. 30-40 mols, of low molecular weight acid for each mol of high molecular weight acid have particular utility for converting synthetic oils of the ester

type into excellent greases. Complex soap proportions of about 5-30 wt. percent, preferably about 8-20 wt. percent, based on total grease may be used in preparing the improved greases of the invention.

To summarize briefly, the instant invention relates to new and improved lubricating grease compositions which have a high degree of storage stability. These novel lubricating greases comprise a lubricating oil, either naturally occurring or synthetic, with a minor but grease thickening amount of a soap-salt complex. This complex comprises the alkaline earth metal soap of a high molecular weight fatty acid having from about 12 to about 30 carbon atoms, preferably about 14 to about 22 carbon atoms, and an alkaline earth metal salt of a low molecular weight fatty acid such as acetic acid, formic acid, furoic acid, propionic acid, acrylic acid, and the like; that is to say, those low molecular weight acids having from about 2 to about 6 carbon atoms. Formic acid and acetic acid salts of alkaline earth metals are preferred. The ratio of the low molecular weight salt to the high molecular weight soap should be within the range of from about 7.5:1 to 20:1, preferably from about 9:1 to 15:1. From about 50 wt. percent to 30.0 wt. percent, preferably from about 8.0 wt. percent to 20.0 wt. percent of the total complex may be used.

Included in the grease formulation, and directly responsible for the high degree of structural stability is a minor but stabilizing amount of an N-acyl p-aminophenol. From about 0.5 wt. percent to about 10.0 wt. percent, based on the weight of the total formulation of the phenol is used, with from 1.0 wt. percent to 6.0 wt. percent being especially preferred. The N-acyl p-aminophenol has the general formula



wherein R is an alkyl group containing from 10 to 22 carbon atoms, preferably 12-18 carbon atoms, and wherein R' and R'' are selected from the group of hydrogen atoms and alkyl groups containing from 1 to 20 carbon atoms, preferably from 3-12 carbon atoms. Especially preferred, and contemplated in the preferred embodiment of the invention, are those N-acyl p-aminophenols according to the general formula above wherein R' and R'' are hydrogen and wherein R is an alkyl group containing from 12 to 18 carbon atoms, such as N-lauroyl p-aminophenol, N-stearoyl p-aminophenol and the like.

It is to be understood, of course, that other commonly known grease additive materials may be incorporated in the greases of invention without departing from the inventive concept. Such materials as tackiness agents, coloring agents, oxidation inhibitors, and the like may be incorporated with the greases as described above with advantage.

What is claimed is:

1. A lubricating grease composition which comprises a major proportion of a lubricating oil and a minor but grease thickening amount of a soap-salt complex, said complex comprising an alkaline earth metal soap of at least one high molecular weight fatty acid with an alkaline earth metal salt of a low molecular weight monocarboxylic acid containing from 2 to 6 carbon atoms, the molar ratio of said salt to said soap in said complex being between about 7.5:1 to 20:1, said lubricating grease composition containing a minor amount sufficient to eliminate crust formation and hardening of a material of the formula



wherein R is an alkyl group of from 10 to 22 carbon atoms and wherein R' and R'' are each selected from the group consisting of hydrogen atoms and alkyl groups containing from 1 to 20 carbon atoms.

2. A lubricating composition according to claim 1 wherein said alkaline earth metal is calcium.

3. A lubricating grease composition according to claim 1 wherein said low molecular weight acid is acetic acid.

4. A lubricating grease composition according to claim 1 wherein R' and R'' of the formula are hydrogen atoms and wherein R of the formula is an alkyl group containing from 12 to 18 carbon atoms.

5. A lubricating grease composition comprising a major proportion of a lubricating oil and a minor but grease thickening amount of a soap-salt complex which comprises the calcium soap of at least one high molecular weight fatty acid having about 12-30 carbon atoms and calcium acetate, the molar ratio of acetic acid radical to high molecular weight fatty acid radical in said complex being between about 7.5:1 to 20:1, said lubricating grease composition containing a minor amount sufficient to eliminate crust formation and hardening of a material of the formula



wherein R is an alkyl group of from 10 to 22 carbon atoms and wherein R' and R'' are each selected from the group consisting of hydrogen atoms and alkyl groups containing from 1 to 20 carbon atoms.

6. A lubricating grease composition according to claim 5 wherein from 8.0 to 20.0 weight percent of the complex is used.

7. A lubricating grease composition according to claim 5 wherein said high molecular weight fatty acid is hydrogenated fish oil acid.

8. A lubricating grease composition according to claim 5 wherein the molar ratio of said acetic acid radical to said fatty acid radical is from 9:1 to 15:1.

9. A lubricating grease composition according to claim 5 wherein R of the formula is an alkyl group of from 12 to 18 carbon atoms and wherein R' and R'' of the formula are hydrogen.

10. A lubricating grease composition which comprises a major proportion of a lubricating oil containing combined therein from about 8.0 weight percent to about 20.0 weight percent, based on the weight of the total composition of a soap-salt complex, said complex comprising calcium acetate and the calcium soap of hydrogenated fish oil acids, the molar ratio of said calcium acetate to said calcium soap being about 9:1 to 15:1, said lubricating grease composition containing about 1.0 weight percent to about 6.0 weight percent of N-lauroyl p-aminophenol.

11. A lubricating grease composition which comprises a major proportion of a lubricating oil containing combined therein from about 8.0 weight percent to about 20.0 weight percent, based on the weight of the total composition of a soap-salt complex, said complex comprising calcium acetate and the calcium soap of hydrogenated fish oil acids, the molar ratio of said calcium acetate to said calcium soap being about 9:1 to 15:1, said lubricating grease composition containing about 1.0 weight percent to about 6.0 weight percent of N-stearoyl p-aminophenol.

12. A method of inhibiting hardening and crust formation of a soap-salt complex thickened grease wherein said complex comprises alkaline earth metal soap of high molecular weight fatty acid and alkaline earth metal salt of C<sub>1</sub> to C<sub>6</sub> fatty acid, the molar ratio of said salt to said soap being about 7.5:1 to 20:1, which comprises

incorporating into said grease about 0.5 to 10.0 wt. percent of a material having the formula:



wherein R is a C<sub>10</sub> to C<sub>22</sub> alkyl group and R' and R'' are selected from the group consisting of hydrogen and C<sub>1</sub> to C<sub>20</sub> alkyl groups.

## References Cited in the file of this patent

## UNITED STATES PATENTS

|   |           |                   |               |
|---|-----------|-------------------|---------------|
| 5 | 2,564,561 | Carmichael et al. | Aug. 14, 1951 |
|   | 2,583,607 | Sirianni et al.   | Jan. 29, 1952 |
|   | 2,618,599 | King et al.       | Nov. 18, 1952 |
|   | 2,625,557 | Cottle et al.     | Jan. 13, 1953 |
|   | 2,629,666 | Morway et al.     | Feb. 24, 1953 |
|   | 2,642,397 | Morway et al.     | June 16, 1953 |